

W. E. GREENAWALT,  
ELECTROLYTIC PROCESS,  
APPLICATION FILED MAR. 22, 1920.

1,373,557.

Patented Apr. 5, 1921.



INVENTOR  
William E. Greenawalt

# UNITED STATES PATENT OFFICE.

WILLIAM E. GREENAWALT, OF DENVER, COLORADO.

## ELECTROLYTIC PROCESS.

1,373,557.

Specification of Letters Patent. Patented Apr. 5, 1921.

Application filed March 22, 1920. Serial No. 367,962.

To all whom it may concern:

Be it known that I, WILLIAM E. GREENAWALT, a citizen of the United States, residing in the city and county of Denver and 5 State of Colorado, have invented certain new and useful Improvements in Electrolytic Processes, of which the following is a specification.

The process relates more particularly to 10 the deposition of metals from impure solutions obtained from leaching ores. It will be described more particularly in its application to copper ores. Its object is to render electrolytic deposition more efficient, and 15 to overcome, or reduce, the effect of the deleterious salts in the solution, during electrolysis. This process may be regarded as a division and a continuation in part, of my co-pending application, Serial No. 66,621, 20 filed December 13, 1915.

The process will be described more particularly in its application to the extraction of copper from its ores, to the conditions of which it is eminently adapted, although it is 25 in no wise intended to limit it to this use alone.

In the electrolysis of impure copper solutions, as for example those obtained from leaching copper ores with a sulfate solution, 30 there is always present iron sulfate, which injuriously affects the operation. Ferrous sulfate in the electrolyte is not particularly harmful, but the ferric sulfate is highly detrimental.

If a solution of copper sulfate, containing ferrous sulfate, is electrolyzed, copper is deposited at the cathode while sulfuric acid and ferric sulfate are produced at the anode, as represented by the following equa- 40 tions:



The ferric sulfate, finding its way to the 45 cathode, combines with the deposited copper and is again reduced to the ferrous condition, thus representing a loss of efficiency, as represented by the equation:



If, however, the ferric sulfate can be reduced at the expense of a comparatively cheap reducing agent, such as sulfur dioxide, then the iron in the electrolyte loses its 55 ability to combine with the deposited copper, while at the same time, an equivalent

of acid is regenerated, as shown by the following equation:



It is not easy to get the results, in practice, indicated by this reaction. The solubility of sulfur dioxide is quite low, and the reaction is too slow to get effective reduction. Even in the presence of an excess of 65 the gas, the ferric salts in the electrolyte will accumulate in highly injurious amounts.

In this process, to more effectively apply 70 the gas, it is first combined with finely divided charcoal. Charcoal, as is well known, absorbs large quantities of sulfur dioxide. How this accomplished is not known, but whether the combination is chemical or physical, is immaterial for the purpose of 75 the present process. It is well known also that charcoal absorbs large quantities of chlorin, and the explanation usually given is, that this is due to the hydrogen and hydrocarbons in the charcoal. Similarly, the 80 reaction of the sulfur gas, as above indicated, may be due to the hydrogen and hydrocarbons in the charcoal, and if the hydrogen and hydrocarbons are replenished as fast as consumed, the same as the sulfur 85 dioxide, the process should be carried out for some time before the beneficial effects of the charcoal are exhausted. The application of sulfur dioxide and charcoal to the treatment 90 of copper ores may be carried out in any suitable apparatus. An apparatus, such as shown in the accompanying drawing, in diagrammatic section, will answer the purpose very well, and serve to more clearly 95 describe the invention.

The accompanying drawing represents a flow sheet, in diagrammatic section, of the preferred method of operating the process, and a suitable apparatus for carrying it out.

Referring to the drawing, 1 shows a leaching vat for applying an acid solution to the ore to dissolve the copper, say, with dilute sulfuric acid. Iron is inevitably dissolved with the copper, and this iron may be in the form of ferrous or ferric sulfate, usually both.

3 is a scrubbing tower, filled with coke or charcoal, and 6 and 15 are agitators containing powdered charcoal, into which the sulfur gas is introduced from the sulfur dioxide generator 19. Its flow is regulated by 110 the valve 18.

The clear copper solution issuing from the vat 1, and regulated by the faucet 2, passes through the scrubbing tower 3, where the excess gas from the agitators 6 and 15 is absorbed by the fresh solution coming from the leaching vat. The solution issues from the tower 3 through the pipe 4, and the excess gas from the agitators enters the tower through the pipe 5. The solution, entering the agitator 6, is thoroughly mixed with the sulfur dioxid in the presence of the finely divided charcoal, and the ferric salts is effectively reduced thereby. The agitator 6 has a rotary member 7, inside, so that the liquid and gas, and charcoal, are brought into intimate contact. The reduced liquid, separated from the charcoal by means of the grating, or filter, 8, issues from the agitator through the outlet 9, and enters the electrolyzer 11, containing the regulation anodes 12, and cathodes 13. When the current is turned on copper is deposited on the cathodes 13, while sulfuric acid and ferric sulfate are produced at the anode 12. The ferric sulfate begins to form as soon as the current is turned on: it is desirable, by regulating the flow, to limit its amount in the cell to from 0.10 per cent. to 0.25 per cent., which amounts are not particularly injurious. From the cell 11, the solution passes through the outlet 14 into the agitator 15, where the ferric salts is again rapidly and completely reduced, as in the agitator 6, and then flows through the outlet of the agitator, 16, into the electrolyzer 22, where the action is the same as in the electrolyzer 11. This cycle is continued until the solution is sufficiently impoverished in copper and regenerated in acid, when it flows through the pipe 23 into the pump 25 and returns to the leaching vat 1 through the pipe line 24. In this way the cycle is repeated indefinitely.

There is a limit to the ability of the charcoal to perform the function, as above described. This is probably due to the exhaustion of the hydrogen, or hydrocarbons in the charcoal. To lengthen the use of the charcoal and to increase its efficiency after exhaustion commences, hydrogen, or a hydrocarbon compound, from the gas generator 21, is introduced into the system with the sulfur dioxid. Its amount is regulated by the valve 20.

55 The process is also applicable to the oxidation of sulfur dioxid to form sulfuric acid.

The concentration of the reducing gas in the electrolyte is an important factor in the reduction of the ferric salts: it is also an important factor in the production of sulfuric acid by the electrolytic oxidation of sulfur dioxid in solution.

The charcoal acts as a concentrator of the gas, probably by occlusion, and this applies to both the sulfur dioxid and to the hy-

drogen or hydrogen containing gas. So far as known, the charcoal itself does not enter into any of the reactions. It acts as an intermediary.

Manifestly other substances besides coke and charcoal may be used for the purpose of concentrating, or occluding, the gas. Coke and charcoal answer the purpose, are cheaply obtainable, and can conveniently be used.

75 I claim:

1. An electrolytic process which consists in treating ores of copper with an acid solution to dissolve the copper, electrolyzing the resulting copper solution containing salts of the variable valent elements to deposit the copper, applying sulfur dioxid as a reducing agent to the electrolyte through the intermediary of finely divided charcoal to reduce the variable valent salts from a higher 80 to a lower valency, and agitating the electrolyte in the presence of the charcoal and the sulfur dioxid.

2. An electrolytic process which consists in treating ores of copper with an acid solution to dissolve the copper, electrolyzing the resulting copper solution containing salts of the variable valent elements to deposit the metal, applying sulfur dioxid to finely divided charcoal and treating the electrolyte therewith to reduce the variable valent salts from a higher to a lower valency.

3. An electrolytic process which consists in treating ores of metals with a solvent for the metals, electrolyzing the resulting metal solution containing salts of the variable valent elements to deposit the metals, agitating the electrolyte in the presence of sulfur dioxid and finely divided charcoal to reduce the variable valent salts in the electrolyte from a higher to a lower valency.

4. An electrolytic process which consists in treating ores of metals with a solvent for the metals, electrolyzing the resulting metal solution containing salts of the variable valent elements to deposit the metals, and treating the electrolyte with sulfur dioxid and a hydrocarbon compound in the presence of charcoal to reduce the variable valent salts in the electrolyte from a higher 110 to a lower valency.

5. An electrolytic process which consists in treating ores of metals with a solvent for the metals, electrolyzing the resulting metal solution containing salts of the variable valent elements to deposit the metals, and treating the electrolyte with sulfur dioxid in the presence of a carbon compound and a hydrogen containing gas to reduce the variable valent salts in the electrolyte from 120 a higher to a lower valency.

6. An electrolytic process which consists in treating ores of metals with a solvent for the metals, electrolyzing the resulting metal solution containing salts of the variable 130

- valent elements to deposit the metals, and  
treating the electrolyte by agitating it in the  
presence of finely divided carbon and a re-  
ducing gas capable of being occluded or con-  
centrated by the divided carbon to reduce  
the variable valent salts from a higher to a  
lower valency.
7. An electrolytic process which consists  
in electrolyzing a liquid and treating the  
electrolyte by agitating it in the presence  
of a gas and a finely divided substance ca-  
pable of concentrating or occluding the gas.
8. An electrolytic process which consists  
in treating ores of copper with an acid solu-  
tin to extract the copper, electrolyzing the  
resulting copper solution containing salts of  
iron to deposit the copper with the simul-  
taneous conversion of the ferrous salts to the  
ferric salts, treating the electrolyte contain-  
ing ferric salts with sulfur dioxide in the  
presence of finely divided carbon and a sub-  
stance capable of promoting the reaction be-  
tween the sulfur dioxide and the ferric salts  
to reduce the ferric salts to the ferrous con-  
dition.
9. An electrolytic process which consists  
in electrolyzing a liquid containing in solu-  
tion substances capable of chemically re-  
acting under the influence of an electric cur-  
rent, confining a gas over the electrolyte,  
and treating the electrolyte with the gas in  
the presence of a substance capable of oc-  
cluding or concentrating the gas in the elec-  
trolyte.
10. An electrolytic process which consists  
in electrolyzing a liquid containing constitu-  
ents capable of reacting with sulfur dioxide  
under the action of an electric current and  
treating the electrolyte with sulfur dioxide in  
the presence of a substance capable of pro-  
moting the reaction.
11. A process which consists in confining  
a gas over a pool of liquid, treating the liq-  
uid of the pool with a gas by associating  
the gas with an insoluble carrier, and elec-  
troyzing the liquid.
12. A process which consists in electro-  
lyzing a liquid containing substances in solu-  
tion which are capable of chemically react-  
ing under the action of an electric current,  
confining a gas over a pool of the liquid,  
treating the liquid of the pool with a gas by  
associating the gas with an insoluble carrier,  
and intimately mixing the gas the carrier  
and the liquid.
13. An electrolytic process which consists  
in confining a gas over a pool of liquid,  
treating the liquid of the pool with the gas  
by associating the gas with an insoluble  
carrier, electrolyzing the liquid treated with  
the gas, and maintaining a flow of liquid  
from the pool to the electrolyzer and from  
the electrolyzer to the pool.
14. An electrolytic process which consists  
in confining a gas over a pool of liquid,  
treating the liquid of the pool with the gas  
in the presence of an insoluble substance  
capable of concentrating or occluding the  
gas, electrolyzing the liquid, and maintain-  
ing a flow of liquid from the electrodes to  
the pool and from the pool to the electrodes,  
and progressively advancing the liquid  
through a series of pools and electrolyzers.

WILLIAM E. GREENAWALT.